

United States Patent [19]  
Kondo et al.

[11] 3,816,116  
[45] June 11, 1974

[54] N-TYPE PHOTORESITIVE MEMBER FOR  
ELECTROPHOTOGRAPHY

[75] Inventors: **Hideyo Kondo**, Tone-machi; **Tatsuo  
Masaki**; **Nobuo Kitajima**, both of  
Tokyo, all of Japan

[73] Assignee: **Canon Kabushiki Kaisha**, Tokyo,  
Japan

[22] Filed: Dec. 23, 1971

[21] Appl. No.: 211,274

[30] Foreign Application Priority Data  
Dec. 29, 1970 Japan..... 45-129134

[52] U.S. Cl..... 96/1.5, 252/501, 75/134 H

[51] Int. Cl..... G03g 5/00

[58] Field of Search..... 96/1 R, 1 PC, 1.5;  
252/501; 75/134 H

[56] References Cited

UNITED STATES PATENTS

2,745,327 5/1956 Mengali ..... 96/1.5

2,803,541 8/1957 Paris ..... 96/1.5  
3,434,832 3/1969 Joseph et al. ..... 96/1.5  
3,655,377 4/1972 Sechak ..... 96/1 PC X  
3,723,105 3/1973 Kitajima et al. ..... 96/1.5 X

FOREIGN PATENTS OR APPLICATIONS

1,135,460 12/1968 Great Britain ..... 96/1.5

OTHER PUBLICATIONS

Keck, "Photoconductivity in Vacuum Coated Selenium Films," J. Optical Soc. Amer., Vol. 42, No. 4, Apr. 1952, pp. 221-225.

Primary Examiner—**Roland E. Martin, Jr.**  
Attorney, Agent, or Firm—**Fitzpatrick, Cella, Harper  
& Scinto**

[57] ABSTRACT

A photosensitive layer for electrophotography is composed of Se-Te alloy containing less than 3 percent by weight of Te and the Te is in a form of selenium-tellurium bond, and the Se-Te alloy has a polarity of N-type.

2 Claims, 1 Drawing Figure

PATENTED JUN 11 1974

3,816,116



## N-TYPE PHOTORESISTIVE MEMBER FOR ELECTROPHOTOGRAPHY

### BACKGROUND OF THE INVENTION

#### 1. Field of the Invention

This invention relates to an N-type photosensitive member comprising Se-Te alloy for electrophotography and a process for preparation thereof.

#### 2. Description of the Prior Art

In general, conventional Se-Te alloy containing a large amount of Te gives a panchromatic photosensitive member of P-type of high sensitivity when vapor deposition of Se-Te alloy is effected by keeping the temperature of a substrate higher than 60°C, particularly, at 65° to 68°C. On the contrary, when the substrate temperature is lower than 60°C, tendency of P-type decreases while tendency of N-type increases and there is produced a thermally unstable and impractical photosensitive member. However, in such a case, there is not obtained a photosensitive member showing N-type only.

A stable and highly sensitive photosensitive member of N-type is very useful, but a method for preparing such photosensitive member is not yet developed.

### SUMMARY OF THE INVENTION

In accordance with the one aspect of the present invention, there is provided a photosensitive layer for electrophotography which comprises Se-Te alloy containing less than 3 percent by weight of Te, the Te being in a form of selenium-tellurium bond, and the Se-Te alloy having a polarity of N-type.

In accordance with another aspect of the present invention, there is provided a photosensitive member for electrophotography comprising a base plate and a photoconductive layer overlying the base plate and composed of Se-Te alloy containing less than 3 percent by weight of Te, the Te being in a form of selenium-tellurium bond and the Se-Te alloy having a polarity of N-type, and if necessary, an insulating layer overlies the photoconductive layer.

In accordance with a further aspect of the present invention, there is provided a process for producing a photosensitive layer for electrophotography which comprises producing a selenium-tellurium alloy containing less than 3 percent by weight of tellurium, containing Se-Te bond and showing N-type polarity by depositing selenium and tellurium on a substrate maintained at a temperature of 60°-70°C.

It is an object of this invention to provide an N-type photosensitive member of excellent durability, good image shapeability, and high sensitivity.

It is another object of this invention to provide a process for producing an Se-Te alloy photosensitive layer for electrophotography of high stability and high sensitivity.

### BRIEF DESCRIPTION OF THE DRAWING

FIG. 1 is a graph showing decay curves for a photosensitive member of the present invention.

### DESCRIPTION OF THE PREFERRED EMBODIMENTS

According to the present invention, an Se-Te alloy photosensitive member of N-type is obtained by adjusting the contents of Te to less than 3 percent by weight.

It has been found that the tellurium contents in an Se-Te alloy affects the polarity (i.e., N-type or P-type) as shown below. At tellurium contents of about 3 percent by weight there appears a boundary. In other words, when the tellurium content exceeds 3 percent, both N-type tendency and P-type tendency coexist, and the higher the tellurium content, the stronger the P-type tendency, and there is not obtained an N-type tendency as desired in the present invention. On the contrary, when the tellurium content is less than 3 percent, the N-type tendency increases and there is obtained an Se-Te alloy photosensitive layer as contemplated in the present invention. Particularly at tellurium content less than 1 percent there appears strong N-type tendency. 15 When the tellurium content becomes less than 0.01 percent, the N-type tendency disappears.

The photosensitive layer is produced by depositing selenium and tellurium on a substrate maintained at a temperature of 60°-70°C to form a selenium-tellurium alloy containing less than 3 percent by weight of tellurium, containing Se-Te bond and showing N-type polarity. When the temperature is higher than 70°C, there occurs crystallization, and when the temperature is lower than 60°C, the resulting Se-Te alloy layer shows 20 both tendencies of N-type and P-type.

For the purpose of the present invention, the tellurium should not be present as an component of a simple mixture of Se and Te, but in a form of Se-Te bond in an Se-Te alloy.

30 In the following cases, the Se-Te alloy shows P-type tendency under the same conditions regardless of the state of materials used for deposition:

1. a commercially available pure selenium is directly deposited;

35 2. a commercially available selenium is melted at 450°C for 3 hours and quenched, and the resulting selenium is deposited;

3. a commercially available selenium is melted at 450°C for 3 hours and cooled gradually to room temperature in a period of 15 hours and the crystalline selenium thus obtained is deposited.

On the other hand, when Te is deposited after Se is deposited, for example, 39.8g. of commercially available selenium is deposited while keeping the substrate temperature at 66°-68°C and then 0.2g. of commercially available tellurium is deposited thereon, or a mixture of 39.9g. of selenium and 0.1g. of tellurium is deposited in a way similar to above, the resulting plate shows low resistance and cannot be used for electrophotography.

As is clear from the above fact, in the Se-Te alloy used in this invention the Te should not be in a form of a simple mixture of Te and Se, but in a form of Se-Te bond. For example, uniform concentration of Te is to be maintained in a process of production of the Se-Te alloy to give Se-Te bond.

The following examples are given for illustrating the present invention, but by no means for restricting the present invention.

### EXAMPLE 1

Fine nine selenium 99.4g. and tellurium 0.6g. were placed in a Pyrex glass tube, and air was evacuated until the pressure became  $10^{-3}$  Torr. and then the tube was sealed. The metals were heated at 550°C for 4 hours with stirring by shaking every 10-15 minutes, then gradually cooled to about 250°C and quenched to

water temperature to produce an alloy. The alloy (40g.) was placed on a vaporizing dish and vapor-deposited on an aluminum substrate to form a deposit layer of about  $50\mu$  thick under the following conditions.

|                             |                          |
|-----------------------------|--------------------------|
| temperature of vapor source | about 300°C              |
| temperature of substrate    | 66-68°C                  |
| vacuum                      | $1 \times 10^{-5}$ Torr. |
| depositing time             | 35 minutes               |

The resulting deposit layer was negatively charged at 1,000 V, imagewise exposed by using an original having light and dark portions at exposure amount of 15 lux. sec. (illuminance, about 40 lux. sec.) and the surface potentials were measured. The result is illustrated in FIG. 1. The curve 1 shows decay at a dark portion and the curve 2 shows decay at a light portion when the photosensitive member is positively charged. The curve 3 shows decay at a dark portion and the curve 4 shows decay at a light portion when the photosensitive member is negatively charged.

As is clear from curve 3 in the graph, when the photosensitive member is negatively charged, decay at a dark portion is very little, and it is clear that there is shown more N-type property.

#### EXAMPLE 2

An Se-Te alloy containing 0.5 percent by weight of Te was used to form a deposit layer in a way similar to Example 1 above. On the resulting Se-Te deposit layer was provided an insulating layer (polyethylene terephthalate film) of about  $30\mu$  thick to produce a photosensitive member. The resulting photosensitive member was subjected to an electrophotographic process as described in U.S. Ser. No. 563,899, filed July 8, 1966.

That is, the photosensitive member was charged (primary charge), imagewise exposed simultaneously discharged by AC, and subjected to blanket irradiation to form electrostatic images. The conditions were as shown below:

|                                                           |                                      |
|-----------------------------------------------------------|--------------------------------------|
| Primary charge                                            | about + 2300V<br>(surface potential) |
| secondary discharging<br>AC voltage<br>exposure amount at | 7500V                                |

|                                                            |               |
|------------------------------------------------------------|---------------|
| light portion<br>exposure amount of<br>blanket irradiation | 15 lux. sec.  |
|                                                            | 150 lux. sec. |

The result is shown below.

|    | Surface potential<br>at light portion (V) | Surface potential<br>at dark portion (V) | Contrast (V) |
|----|-------------------------------------------|------------------------------------------|--------------|
| 10 | + 750                                     | 0                                        | 750          |

#### EXAMPLE 3

The procedures of Example 2 were followed except employing corona discharge of polarity opposite to that of the primary charging in place of AC discharging. The conditions were as shown below:

|                                                              |                                      |
|--------------------------------------------------------------|--------------------------------------|
| primary charge                                               | about + 2300V<br>(surface potential) |
| secondary discharging<br>exposure amount at<br>light portion | - 7500V                              |
| exposure amount of blanket<br>irradiation                    | 15 lux. sec.                         |
|                                                              | 150 lux. sec.                        |

|    | Surface potential<br>at light portion (V) | Surface potential<br>at dark portion (V) | Contrast (V) |
|----|-------------------------------------------|------------------------------------------|--------------|
| 30 | + 300                                     | - 500                                    | 800          |

We claim:

1. Process for producing a photosensitive layer for electrophotography which comprises producing a selenium-tellurium alloy containing more than 0.01 percent and less than 3 percent by weight of tellurium, containing Se-Te bond and showing N-type polarity by heating for a period of time sufficient to produce a Se-Te chemical bond and subsequently vapor depositing said selenium and tellurium alloy on a substrate maintained at a temperature of 60°-70°C.

2. A photosensitive member comprising the photosensitive layer prepared according to claim 1 and an insulating layer overlaying the photosensitive layer.

\* \* \* \* \*